



L. F. ROBERTSON, OF MORRISANIA, NEW YORK.

*Letters Patent No. 87,202, dated February 23, 1869.*

**IMPROVED COMPOUND FOR BATING HIDES AND SKINS.**

The Schedule referred to in these Letters Patent and making part of the same.

*To all whom it may concern:*

Be it known that I, L. F. ROBERTSON, of Morrisania, in the county of Westchester, State of New York, have invented a new and improved Compound for Bating Hides and Skins; and I do hereby declare the following to be a full, clear, and exact description thereof, which will enable those skilled in the art to make and use the same.

This invention relates to a compound for bathing all sorts of hides and skins, for upper and harness-leather, and also sheep and goat-skins, said compound being made of water, molasses, sawdust, and urine, or, instead of sawdust, blood may be used.

These ingredients are mixed together, in about the following proportions:

Water, two hundred gallons; molasses, one gallon; sawdust, one and a half bushel; filtered urine, two and a half gallons. Or, instead of this, water, two hundred gallons; molasses, one gallon; blood, one gallon; filtered urine, two and a half gallons.

These proportions will, however, undergo slight modifications, according to the condition of the water, and of the season; and for various kinds of hides and skins the proportions must be increased or diminished.

My bathing-compound works fully as good as the bates, pures, or drenches, which are at present in general use, and which are made of flour, or bran, or of dung of chickens, pigeons, or dogs, or diluted muriatic acid.

The peculiar advantages of my bathing-compound, when compared with the bates previously used, may be enumerated as follows:

First, by the application of my compound, any common workman is enabled to perform the bathing-process, without danger of injuring or spoiling the stock, which often happens by the old bathing-process, even if an experienced workman has charge of the labor.

Second, the cost of my process is only about one-tenth of that of the old process.

Third, my process is not subjected to the influence of thunder-storms, whereby the stock subjected to the old bathing-process is many times damaged or spoiled.

Having thus described my invention,

What I claim as new, and desire to secure by Letters Patent, is—

A compound for bathing hides and skins, made of urine, molasses, sawdust, and water, mixed together, substantially in the manner herein set forth.

Also, a compound for bathing hides and skins, made of urine, molasses, blood, and water, mixed together, substantially in the manner herein specified.

This specification signed by me, this 28th day of December, 1868.

L. F. ROBERTSON.

Witnesses:

W. HAUFF,  
ERNEST F. KASTENHUBER.